

## UNITED STATES PATENT OFFICE

GUSTAV REDDELLEN AND WERNER MÜLLER, OF LEIPZIG, GERMANY, ASSIGNEES, BY  
MESNE ASSIGNMENTS, TO AGFA ANSCO CORPORATION, OF BINGHAMTON, NEW  
YORK, A CORPORATION OF NEW YORK

PROCESS OF DEVELOPING PHOTOGRAPHIC MATERIALS AND NEW PHOTOGRAPHIC  
DEVELOPERS

No Drawing. Application filed November 2, 1927, Serial No. 230,687, and in Germany November 19, 1926.

The present invention relates to a process of developing photographic materials and to new photographic developers, more particularly to the photographic developers comprising as developing agent a compound of the general formula:



10 wherein X represents hydrogen or the group —CH<sub>2</sub>.CH<sub>2</sub>.OH.

It is known that 4-amino-1-hydroxybenzene and its N-mono-alkylated derivatives are developers of the latent photographic image in silver halide layers. Of the twice 15 N-substituted 4-amino-1-hydroxybenzenes only 4-hydroxyphenyl-N-alkylglycines have hitherto been known as photographic developers.

20 Now we have found that the 4-hydroxyethylamino-1-hydroxybenzene and the 4-dihydroxyethylamino-1-hydroxybenzene are particularly suited for the use as photographic developers. Both compounds were hitherto unknown, the manufacture of them 25 has been described in our Patent Number 1,712,716, dated May 14, 1929, and consists in the condensation of 4-amino-1-hydroxybenzene with a halogenhydrin of glycol.

30 A suitable developer consists of a solution of 1 gram of 4-dihydroxyethylamino-1-hydroxybenzene in 200 cc. of water with 10 grams of crystallized sodium sulphite, 10 grams of potassium carbonate and 0.05 gram 35 of potassium bromide. It develops just as a developer does from 4-amino-1-hydroxybenzene as developing agent but it is of more advantageous composition and of normal concentration. The chief advantage is that 40 the new developing agent is permanent in solid condition and has an essentially greater stability in the alkaline developing solution than 4-amino-1-hydroxybenzene has. For the developing solution made from 4-amino-1-hydroxybenzene rapidly becomes dark in 45 the air, whereas the developing solution made from 4-dihydroxyethylamino-1-hydroxybenzene remains unchanged for days.

A solution of 1 gram of the sulphate of 50 4-hydroxyethylamino-1-hydroxybenzene in

200 cc. of water with 20 grams of crystallized sodium sulphite and 5 grams of potassium carbonate develops more strongly than those made from normal 4-amino-1-hydroxybenzene developers. The new developer excels the best of the hitherto known developers in that it is extraordinarily soluble, is remarkably permanent even in alkaline solutions and, what is of particular advantage, develops completely without fog, even in solution free from potassium bromide.

55 What we claim is:

1. A photographic developer containing together with other developer ingredients a compound of the general formula:



60 wherein X represents a substituent of the group consisting of

70 —H and —CH<sub>2</sub>.CH<sub>2</sub>.OH.

2. A photographic developer containing together with other developer ingredients 75 4-hydroxyethylamino-1-hydroxybenzene.

3. A photographic developer comprising sodium sulfite and a compound of the general formula:



80 wherein X represents a substituent of the group consisting of

85 —H and —CH<sub>2</sub>.CH<sub>2</sub>.OH.

4. A photographic developer comprising sodium sulfite and 4-hydroxyethylamino-1-hydroxybenzene.

5. A photographic developer comprising an alkaline solution containing sodium sulfite 90 and a compound of the general formula:



95 wherein X represents a substituent of the group consisting of

—H and —CH<sub>2</sub>.CH<sub>2</sub>.OH.

100 6. A photographic developer comprising an alkaline solution containing sodium sul-

fite and 4-hydroxyethylamino-1-hydroxybenzene.

7. A photographic developer comprising sodium sulfite, potassium carbonate and a compound of the general formula:



wherein X represents a substituent of the group consisting of

—H and —CH<sub>2</sub>CH<sub>2</sub>OH.

8. A photographic developer comprising sodium sulfite, potassium carbonate and 4-hydroxyethylamino-1-hydroxybenzene.

15 9. A photographic developer comprising sodium sulfite, potassium carbonate, potassium bromide and a compound of the general formula:



wherein X represents a substituent of the group consisting of

25 —H and —CH<sub>2</sub>CH<sub>2</sub>OH.

10. A photographic developer comprising sodium sulfite, potassium carbonate, potassium bromide and 4-hydroxyethylamino-1-hydroxybenzene.

30 11. The process of developing photographic materials which comprises treating the same with a solution containing a compound of the general formula:



wherein X represents a substituent of the group consisting of

40 —H and —CH<sub>2</sub>CH<sub>2</sub>OH.

12. The process of developing photographic materials which comprises treating the same with a solution containing 4-hydroxyethylamino-1-hydroxybenzene.

45 13. The process of developing photographic materials which comprises treating the same with a solution containing together with other developer ingredients a compound of the general formula:



wherein X represents a substituent of the group consisting of

55 —H and —CH<sub>2</sub>CH<sub>2</sub>OH.

14. The process of developing photographic materials which comprises treating the same with a solution containing together with other developer ingredients 4-hydroxyethylamino-1-hydroxybenzene.

60 15. The process of developing photographic materials which comprises treating the same with a solution containing sodium

sulfite and a compound of the general formula:



70 wherein X represents a substituent of the group consisting of —H and —CH<sub>2</sub>CH<sub>2</sub>OH.

16. The process of developing photographic materials which comprises treating the same with a solution containing sodium sulfite and 4-hydroxyethylamino-1-hydroxybenzene.

75 17. The process of developing photographic materials which comprises treating the same with an alkaline solution containing sodium sulfite and a compound of the general formula:



80 wherein X represents a substituent of the group consisting of —H and —CH<sub>2</sub>CH<sub>2</sub>OH.

18. The process of developing photographic materials which comprises treating the same with an alkaline solution containing sodium sulfite and 4-hydroxyethylamino-1-hydroxybenzene.

85 19. The process of developing photographic materials which comprises treating the same with a solution containing sodium sulfite, potassium carbonate and a compound of the general formula:



90 wherein X represents a substituent of the group consisting of

—H and —CH<sub>2</sub>CH<sub>2</sub>OH.

95 20. The process of developing photographic materials which comprises treating the same with a solution containing sodium sulfite, potassium carbonate and 4-hydroxyethylamino-1-hydroxybenzene.

100 21. The process of developing photographic materials which comprises treating the same with a solution containing sodium sulfite, potassium carbonate, potassium bromide and a compound of the general formula:



105 wherein X represents a substituent of the group consisting of

—H and —CH<sub>2</sub>CH<sub>2</sub>OH.

110 22. The process of developing photographic materials which comprises treating the same with a solution containing sodium sulfite, potassium carbonate, potassium bromide and 4-hydroxyethylamino-1-hydroxybenzene.

115 In testimony whereof, we affix our signatures.

GUSTAV REDDELLEN.  
WERNER MÜLLER.